

July 6, 1937.

O. R. RICE

2,085,925

TUYÈRE

Filed Oct. 22, 1934

2 Sheets-Sheet 1



Fig. 7



Fig. 8



Fig. 9



Fig. 1



Fig. 6



Fig. 2



Fig. 3



Fig. 4



Fig. 5

Inventor  
Owen R. Rice.

By: Wilkinson, Hugley, Bryan & Knight  
Atty's.

July 6, 1937.

O. R. RICE

2,085,925

TUYÈRE

Filed Oct. 22, 1934

2 Sheets-Sheet 2



Fig. 10



Fig. 11



Fig. 13



Fig. 12

Fig. 14

Inventor  
Owen R. Rice.  
By Wilkinson Huxley Byron & Knight  
Atty's.

## UNITED STATES PATENT OFFICE

2,085,925

## TUYÈRE

Owen E. Rice, Chicago, Ill., assignor to Freyn Engineering Company, Chicago, Ill., a corporation of Maine

Application October 22, 1934, Serial No. 749,371

4 Claims. (Cl. 122—6.6)

The present invention relates to improvements in tuyères.

More particularly the present invention relates to fluid cooled tuyères having refractory 5 noses.

An object of the present invention is to provide an improved tuyère which will stand up well under the severe conditions encountered in furnaces.

10 A further object is to provide a tuyère having a refractory nose composed of a material similar to that deposited within a blast furnace in service to accomplish the result that said nose will effectually resist both oxidizing and reducing conditions which may exist in the vicinity of the tuyère.

A further object is to simplify the manufacture of tuyères having preformed refractory blocks in the noses thereof.

20 A further object is to provide an improved method of making a tuyère embodying preformed refractory blocks in the nose thereof.

Further objects will appear as the description proceeds.

25 Referring to the drawings—

Figure 1 is a view in end elevation showing the nose portion of a tuyère embodying the principles of the present invention, illustrating particularly the disposition of refractory blocks 30 within the nose portion of the tuyère;

Figure 2 is a fragmentary sectional view taken along the plane indicated by the arrows 2—2 of Figure 1;

35 Figure 3 is a view similar to Figure 2 but showing an alternative construction for holding the refractory blocks in place;

Figures 4 and 5 are views in end elevation and side elevation, respectively, of the block appearing in Figure 2;

40 Figure 6 is a view in end elevation of the block appearing in Figure 3;

Figure 7 is a fragmentary view similar to Figure 1 but showing the arrangement of preformed refractory blocks for a different diameter of tuyère;

Figure 8 shows the arrangement of blocks for another diameter of tuyère;

Figure 9 shows the arrangement of blocks for 50 another diameter of tuyère;

Figure 10 shows the arrangement of blocks for still another diameter of tuyère;

Figure 11 illustrates the method of spacing the refractory blocks preparatory to the operation of casting the tuyère;

Figure 12 is a fragmentary elevational view of the structure shown in Fig. 11;

Figure 13 is a view illustrating how a portion of a shim may remain after the casting operation; and

Figure 14 is a fragmentary elevational view of the structure shown in Figure 13.

The present invention has been illustrated in connection with a tuyère of the type generally known as water-cooled. By reference to Figure 2 it will be noted that the tuyère comprises the inner cone wall 10, the outer cone wall 11, and the front wall 12. Said walls, together with a back wall (not illustrated), form a jacket for cooling medium, usually water, through which the cooling medium may flow in a continuous stream to carry away heat from the metal of the tuyère.

Extending forwardly from the front wall 12 are the inner annular rib or fin 13 and the outer annular rib or fin 14, which ribs or fins 13 and 14 are disposed coaxially of the tuyère. In the outwardly opening recess between the front wall 12 and the annular ribs 13 and 14 are a plurality of preformed segmental blocks 15—15, which blocks, in order that they may fit approximately around the circumference of a circle, have side faces tapering toward one another.

In the manufacture of a tuyère embodying the principles of the present invention, the copper of the tuyère is cast around the preformed refractory blocks 15—15. According to the construction illustrated in Figure 2, a dove-tailed tenon 16 is provided, which tenon extends circumferentially of the tuyère in the space provided by the wall 12 and the annular ribs or fins 13 and 14.

In the construction illustrated in Figure 3, the faces of the refractory blocks 15—15, which face the base of the tuyère, are provided with a pair of holes 17—17. These holes are disposed at an angle one to the other so that when they are filled up with copper in the casting operation to form lugs, indicated by the numerals 17a—17a, 45 the blocks are held firmly in a manner comparable to the "toe-nailing" of a board. In either of the constructions illustrated in Figures 2 and 3, the copper side walls or ribs 13 and 14 may burn away in service, but the blocks are securely 50 held either by the tenon 16 or the lugs 17a—17a within the holes 17—17, which tenons or lugs are themselves an intimate part of the cool water wall of the tuyère body. In the construction illustrated in Figure 3, a vent 18 is provided com- 55

municating with each pair of holes 17-17, whereby to facilitate the casting operation.

In the zone of the tuyères in a blast furnace there is present a highly scorifying fluid slag which will flux with substances which are metallurgically either acid, such as silica, or basic, such as lime, or even neutral, such as alumina. Even the brickwork, which consists chiefly of some of these materials, is not resistant to this slag. The atmosphere in this zone of the furnace is prevailingly reducing, so that certain so-called refractories consisting of metallic oxides, such as chromic oxide, cannot endure in this atmosphere. There are times also when, locally, the atmosphere is highly oxidizing. Ordinary carbon, sometimes regarded as a refractory, is far from proof against this condition.

According to the present invention, it is contemplated to use a substance such as is formed in the operation of a blast furnace. The furnace-born substance referred to is graphite. Early in the operation of the furnace, graphite deposits naturally upon the brick walls of the hearth and the lower bosh, this deposit being in the form of a heavy coating of laminated crystalline graphite. This graphite is produced by precipitation from the molten pig iron, which is really a super-saturated solution of carbon in iron. It protects the brick against the fluxing action of the slag and the high temperature. It is itself unaffected by a reducing atmosphere. It is only very difficultly oxidizable. It is impervious to the molten pig iron, of which it is really a product. It is the natural protective material in the furnace. It appears to be the only universal refractory in the blast furnace sense. Without its protection the brick structure would not survive.

The present invention therefore contemplates the use of crystalline graphite in the tuyère nose as a protective agent. In casting copper about a preformed rigid core of graphite, difficulty will be encountered due to the tendency of the copper to split upon cooling. This is because the coefficient of expansion of copper is higher than that of crystalline graphite. Moreover, since tuyères are made in many sizes, it would be necessary to have on hand many sizes of crystalline graphite cores. In order to simplify the matter of stocking cores, and for the further purpose of overcoming the difficulty of splitting of the copper upon cooling, the present invention contemplates the use of a plurality of segmental preformed blocks which can be disposed circularly to form a core of any preferred diameter, within limits. Figure 1 shows a core made up of nine full blocks 15 and one cut block, the cut block being indicated by the numeral 19. In the operation of casting the tuyère, shims 20-20 (Fig. 11) of volatile substance, such as wood or paper, may be

located between the blocks to permit the copper to contract upon cooling. The fact that the adjacent sides of the blocks do not make flat contact in certain cases is of no consequence. These spaces will be filled with intrusions or fins of cast copper, indicated by the numerals 21-21 (Fig. 13), which will serve the better to hold the blocks in place. In case the shims are not completely volatilized, no harm will result. Fragments of such shims are indicated by the numerals 10 20a-20a in Figure 13.

Figures 7, 8, 9 and 10 indicate relative positions of blocks such as shown in Figure 1, but for tuyères of different diameters.

The present invention has the advantage that 15 the nose of the tuyère is protected by a refractory such as is a result of the furnace operation and therefore is immune to the destructive forces within the furnace. By reason of the fact that the refractory is cast within the tuyère in the 20 form of a plurality of preformed blocks, it is a simple matter to provide for the casting of different sizes of tuyères as required, and, further, it is a simple matter to provide for the differences 25 in the co-efficient of expansion of the copper and the blocks, whereby the blocks may move in the cooling operation to allow contraction of the copper while cooling, whereby to avoid splitting of the copper.

The present disclosure is of course subject to 30 modification. It is intended to cover all such modifications that fall within the scope of the appended claims.

What is claimed is—

1. A blast furnace tuyère having an annular water jacket in the body portion thereof and a nose portion of crystalline graphite.
2. A blast furnace tuyère comprising a metallic body having a cooling chamber formed therein and having a nose portion including a plurality of imperforate annular fins with an open space between them extending beyond the end of said cooling chamber, and a set of preformed circularly disposed graphite blocks disposed between said fins and keyed to said body portion.
3. A blast furnace tuyère comprising a metallic body having a cooling chamber formed therein and having a nose portion including a plurality of imperforate annular fins with an open space between them extending beyond the end of said cooling chamber, and a set of preformed circularly disposed refractory blocks disposed between said fins and keyed to said body portion.
4. An assembly of elements for the manufacture of a tuyère comprising a plurality of circularly disposed refractory blocks and members of volatile material for spacing said blocks apart circumferentially.

OWEN R. RICE.